

**1****3,560,610****HAIR-SETTING COMPOSITION**

Maria A. Korden, Fairfax, Del., assignor to  
Hercules Incorporated, Wilmington, Del.  
No Drawing. Filed Oct. 13, 1967, Ser. No. 675,022  
Int. Cl. A61k 7/10

U.S. Cl. 424—72

7 Claims

**ABSTRACT OF THE DISCLOSURE**

A hair-setting lotion is provided which is comprised of an aqueous solution of a reaction product of a water-soluble polyaminoureylene-epichlorohydrin resin and a water-soluble material such as sodium sulfite.

This invention relates to novel hair-setting compositions or lotions and to their use in setting hair.

Two primary methods are employed in the art of hair dressing. In one of these, called "permanent waving," the configuration of individual hair fibers is substantially permanently changed to impart a curl or wave to the hair. A permanent waving process involves the use of chemical agents which react with the material of the hair fibers to soften and/or change it chemically in order to achieve a desired permanently waved configuration. This process can be carried out either at approximately room temperature, the process then being called "cold permanent waving," or at an elevated temperature.

The second process involved in hair dressing is that of setting the hair; that is, imparting to the hair a temporary set or temporarily changed configuration for the purpose of obtaining a particular hair style. This temporary set is changed whenever the hair style is changed. The hair-setting process can also be carried out either at room temperature or at elevated temperature, and in the past there have been employed certain water-soluble gums and resins for imparting a temporary set to hair.

In the case of permanently waved hair the curl or wave in the hair remains substantially unaltered for the remainder of the life of the hair under ordinary conditions. A hair set, however, is not permanent but is generally removed by wetting the hair with water. Usually, the hair set is removed by shampooing the hair with mild shampoo.

The present invention is directed to a novel hair-setting composition for use in imparting a temporary set to hair.

In accordance with this invention there is provided a novel hair-setting composition comprised of an aqueous solution of a water-soluble resinous material. The hair-setting composition of this invention can be used to impart a highly satisfactory temporary set to hair which has good resistance to high humidity. The hair-setting composition is applied to water-damp hair, usually in the form of a fine spray, and the thus treated hair is set to a desired configuration usually by use of rollers. The treated hair is subsequently dried. The water-soluble resinous material deposited on the hair provides the desired set-holding characteristics until removed. The deposited resinous material is essentially tack free and remains so even when the hair is exposed to conditions of high humidity. The resinous material deposited on the hair can be easily and readily removed, despite its resistance to humid conditions, by washing with a mild shampoo whereby the hair-set is removed and the hair can be reset and restyled, if desired.

The water-soluble resinous material of this invention is the reaction product derived by reaction of (1) a water-soluble polyaminoureylene-epichlorohydrin resin, and (2) a water-soluble material selected from the group consisting of (a) water-soluble sulfites; (b) water-soluble

**2**

bisulfites; (c) water-soluble thiosulfates; (d) water-soluble thioglycolates; and (e) mixtures of two or more. The hair-setting compositions of this invention are essentially free of sulfite anions, bisulfite anions, thiosulfate anions, and thioglycolate anions.

The amount of water-soluble material (2) used in carrying out the reaction to provide the water-soluble resinous material of this invention will be that which will provide from about 0.2 mole to 1.0 mole, and preferably from about 0.5 mole to 0.9 mole, of sulfite anion, bisulfite anion, thiosulfate anion, or thioglycolate anion per mole of epichlorohydrin moiety of the water-soluble polyaminoureylene-epichlorohydrin resin (1). Reaction is carried out in aqueous media at a pH of about 4.5 to 15 about 11, preferably at a pH of from about 6 to about 8.5, and at a temperature of from about 25° C. to about 100° C. for a period of time of from about 1/2 hour to 2 weeks, or longer if required. Preferred temperature range is from about 25° C. to about 80° C. Reaction 20 time varies inversely with temperature. Reaction is carried out until essentially all bisulfite anion, sulfite anion, thiosulfate anion, and/or thioglycolate anion has reacted and there is less than about 0.15% anion present in the solution. After reaction, the solution is adjusted to a 25 desired solids concentration and to a pH of from about 6 to about 7.5.

Examples of suitable water-soluble sulfites for use herein include sodium sulfite, potassium sulfite, and ammonium sulfite. Examples of suitable water-soluble bisulfites for use in this invention include sodium bisulfite, potassium bisulfite, ammonium bisulfite, sodium metabisulfite, potassium metabisulfite, and ammonium metabisulfite. Examples of water-soluble thiosulfates include sodium thiosulfate, potassium thiosulfate, and ammonium thiosulfate. Examples of water-soluble thioglycolates include sodium thioglycolate, potassium thioglycolate, and ammonium thioglycolate. Mixtures of two or more of the above can be used if desired.

Water-soluble polyaminoureylene-epichlorohydrin resins (1) employed herein are water-soluble polymeric reaction products of epichlorohydrin and a water-soluble polyaminoureylene containing tertiary amino nitrogens.

The polyaminoureylene is water-soluble and is derived by reaction of urea and a polyalkylene polyamine containing at least three amine groups, at least one of which is a tertiary amine group in a mole ratio of polyalkylene polyamine to urea of from about 0.7:1 to about 1.5:1. The reaction can, if desired, be carried out in a suitable organic diluent such as xylene. The reaction is carried 50 out preferably in aqueous media.

The polyalkylenepolyamine reactant will have at least three amine groups, at least one of which is a tertiary amine group. Examples of suitable polyalkylene polyamines include methyl bis(3 - aminopropyl)amine, methyl bis(2 - aminoethyl)amine, 4,7 - dimethyltriethylenetetraamine and the like. Mixtures of two or more can be employed if desired.

Temperature employed in carrying out reaction between urea and polyalkylene polyamine can vary from about 125° C. to about 250° C. at atmospheric pressure. Temperatures between about 175° C. and about 225° C. are preferred. The time of reaction will vary depending upon temperature, but will usually be from about 1/2 hour to about 4 hours. Reaction time varies inversely with temperature. In any event, reaction is continued to substantial completion.

In carrying out reaction between urea and polyalkylene polyamine, it is preferred to use a mole ratio of polyalkylenepolyamine to urea of about 1:1. However, as above set forth, mole ratios from about 0.7:1 to about 1.5:1 can be used.

Reaction of the polyaminoureylene with epichlorohydrin is carried out at a temperature of from about 25° C. to about 80° C., and preferably at a temperature of from about 35° C. to about 50° C., until the viscosity of a 25% solids solution in water at 25° C. has reached about B or higher on the Gardner-Holdt scale. This reaction is preferably carried out in aqueous solution at solids concentrations from about 20% to about 50% to moderate the reaction. The reaction can also be moderated by decreasing the pH of the aqueous polyaminoureylene solution with acid prior to addition of epichlorohydrin or immediately after the addition of epichlorohydrin. This adjustment is usually made to pH 8.5-9.5 but may be made to as low as pH 7.5 in some cases with quite satisfactory results. When the desired viscosity is reached, the product is cooled to about 25° C.

In the polyaminoureylene-epichlorohydrin reaction, it is preferred to use a mole ratio of epichlorohydrin to free amine groups in the polyaminoureylene of from about 1.0:1 to about 1.7:1. Satisfactory results can be obtained employing from about 0.8 mole to about 2.0 moles of epichlorohydrin for each free amine group of the polyaminoureylene.

The following examples are illustrative of the invention. All parts and percentages are by weight unless otherwise specified.

#### EXAMPLE 1

To a resin kettle are charged 217.5 parts of methyl bis(3-aminopropyl)amine and 90 parts of urea. The resulting mixture is heated at about 180° C. for about 45 minutes, and is then diluted with about 300 parts water and cooled. The resulting polyaminoureylene has an intrinsic viscosity of about 0.20 and a total solids content of about 40%. 212 parts of the above polyaminoureylene solution containing 85.5 parts solids is diluted with 233 parts of water and acidified with 14.1 parts of concentrated hydrochloric acid. The resulting solution is then treated with 69.4 parts of epichlorohydrin and heated to 40-55° C. until the Gardner-Holdt viscosity reaches K. The resulting solution is acidified to a pH of about 2 with concentrated HCl and heated to about 65° C. for about 1.5 hours while maintaining the pH of about 2 by periodic additions of concentrated HCl. The resulting solution after cooling contains about 28% total solids. To 50 parts of the above resin solution are added about 150 parts of water and 3.48 parts of sodium metabisulfite. The pH is adjusted to about 8.2 with sodium hydroxide solution and water is added to a total weight of mixture about 400 parts to provide a hair-setting lotion.

#### EXAMPLE 2

A strand or tress of hair, 10 inches long and weighing 1 gram, is dampened with water. It is then sprayed with the hair-setting lotion of Example 1. The treated tress is rolled up on rollers, dried with a home-type hair dryer and combed out. The curl length is about 3.41 inches. The curled tress is hung in a high humidity chamber (75° F., 75% R.H.). After two hours exposure, the length of the curled tress is about 6.7 inches.

#### EXAMPLE 3

To 212 parts of an aqueous solution of polyaminoureylene (40.3% solids) is added 233 parts water. The pH of the solution is adjusted to 9.6 by addition of concentrated HCl. The polyaminoureylene is the condensation product of about 1 mole of urea and about 1 mole of methyl bis(3-aminopropyl)amine. To the resulting mixture there is added 69.4 parts of epichlorohydrin. This mixture is then heated at 40° C. for about 2½ hours and then at 50° C. for about ½ hour. At the end of this time the reaction mass has a Gardner-Holdt viscosity of L and a pH of 8.5. The reaction mass is cooled to about 40° C. and the pH thereof is adjusted to 8.25 by addition of HCl. A solution of 40.2 parts of sodium metabisulfite dissolved in 100 parts water is added followed by addition

of 100 parts water. The temperature of this reaction mass increases to about 50° C. in about ½ hour and then decreases to about 40° C. in about ¾ hour. The 40° C. temperature is maintained for an additional 2½ hours. At the end of this period the sulfite anion concentration, calculated as NaHSO<sub>3</sub> is less than 0.1%. The reaction mass is diluted with 3,312 parts water to provide a solution having a solids content of about 4.3% and a pH of about 7.1.

#### EXAMPLE 4

The solution of Example 3 is tested as a hair-set lotion in accordance with the procedure of Example 2. Curled tress length after treatment and combing is 4.2 inches and 6.6 inches after being subjected to 75° F., 75% R.H. for 2 hours. Water treatment, used as a control, gives a curled tress of 4.8 inches after combing and a tress having a length of 7.8 inches after being subjected to 75° F., 75% R.H. for 2 hours.

#### EXAMPLE 5

Example 3 is repeated using ammonium thioglycolate instead of sodium metabisulfite to provide an equally satisfactory hair-set lotion.

#### EXAMPLE 6

Example 3 is repeated using sodium thiosulfate pentahydrate instead of sodium metabisulfite to provide an equally satisfactory hair-set lotion.

Thus, in accordance with this invention, there is provided a novel hair-setting composition that can be employed to impart a temporary set to hair which has good set-holding properties when exposed to conditions of high humidity.

The amount of resinous material in the hair-setting composition is from about 0.5% to 10%, by weight of the total weight of the composition, and preferably from about 1½% to about 5½% by weight. Lower concentrations can be employed; however, they are not so desirable because excessively large quantities of the composition must be applied to the hair in order to obtain an adequate application of resinous material. Higher concentrations are undesirable because of the tendency to apply more resinous material to the hair than is needed. The pH of the hair-setting compositions preferably will be from about 6 to about 7.5. Required pH adjustments in this invention can be made by use of either dilute sulfuric acid or dilute sodium hydroxide.

The hair-setting composition of this invention can be applied to the hair in any convenient manner such as, for example, by means of a spray pump.

Additives often used in hair-setting compositions can also be incorporated into the compositions of this invention, if desired. Thus, for example, glycerine and/or water-soluble lanolin derivatives, such as ethoxylated lanolin, can be added to improve sheen or luster of treated hair. Water-soluble dyes can be added as well as perfumes and the like.

It is to be understood that the above description and examples are illustrative of this invention and not in limitation thereof.

What I claim and desire to protect by Letters Patent is:

1. A hair-setting lotion comprising an aqueous solution containing, by weight, from about 0.5% to about 10% of a reaction product of (1) a water-soluble polyaminoureylene-epichlorohydrin resin derived by reacting epichlorohydrin and a water-soluble polyaminoureylene containing tertiary amino nitrogens in a mole ratio of epichlorohydrin to free amine groups in the polyaminoureylene of from about 1.0:1 to about 1.7:1, and polyaminoureylene being derived by reaction of urea and a polyalkylene polyamine containing at least three amine groups, at least one of which is a tertiary amine group, in a mole ratio of polyalkylene polyamine to urea of from about 0.7:1 to about 1.5:1, said polyalkylene polyamine being selected from the group consisting of methyl bis(3-

aminopropyl)amine, methyl bis(2-aminoethyl)amine, 4,7-dimethyltriethylenetetramine, and mixtures thereof and (2) a water-soluble material selected from the group consisting of sodium, potassium, and ammonium sulfites, bisulfites, thiosulfates, and thioglycolates and mixtures thereof, the amount of water-soluble material (2) used to prepare the reaction product being that which will provide from about 0.2 mole to 1.0 mole of sulfite anion, bisulfite anion, thiosulfate anion, thioglycolate anion, or mixtures thereof per mole of epichlorohydrin moiety of the water - soluble polyaminoureylene - epichlorohydrin resin, said reaction product being derived by reaction of the water - soluble polyaminoureylene - epichlorohydrin resin (1) and water-soluble material (2) in aqueous media at a pH of about 4.5 to about 11 and at a temperature of from about 25° C. to about 100° C. until essentially all bisulfite anion, sulfite anion, thiosulfate anion, thioglycolate anion, or mixtures thereof has reacted and there is less than 0.15% anion present.

2. The hair-setting lotion of claim 1 wherein the pH of the aqueous solution is from about 6 to about 7.5.

3. The hair-setting lotion of claim 1 wherein the polyaminoureylene is derived by reaction of urea and methyl bis(3-aminopropyl)amine.

4. The hair-setting lotion of claim 1 wherein the amount of water-soluble material (2) used is that which will pro-

vide from about 0.5 mole to about 0.9 mole of the anion of the water-soluble material per mole of epichlorohydrin moiety.

5. The hair-setting lotion of claim 4 wherein the pH of the aqueous solution is from about 6 to about 7.5.

6. The hair-setting lotion of claim 4 wherein the polyaminoureylene is derived by reaction of urea and methyl bis(3-aminopropyl)amine.

7. In the method of providing a temporary wave set to hair wherein there is applied to water-damp hair a hair-setting lotion, the thus treated hair being subsequently styled to a desired configuration, the improvement wherein the hair-setting lotion employed is the hair-setting lotion of claim 1.

#### References Cited

##### UNITED STATES PATENTS

|           |        |                   |        |
|-----------|--------|-------------------|--------|
| 3,141,825 | 7/1964 | Goldemberg et al. | 424—72 |
| 3,250,682 | 5/1966 | Wilmsmann et al.  | 424—71 |
| 3,262,917 | 7/1966 | Maeder            | 424—71 |

ALBERT T. MEYERS, Primary Examiner

F. E. WADDELL, Assistant Examiner

U.S. Cl. X.R.

132—7; 424—71